

# United States Patent

Brown

[15] 3,679,719

[45] July 25, 1972

[54] **NON-YELLOWING SOFTENING AGENT FOR COTTON AND RAYON TEXTILES**

[72] Inventor: **James Marvin Brown**, Charlotte, N.C.

[73] Assignee: **American Cyanamid Company**, Stamford, Conn.

[22] Filed: **March 12, 1970**

[21] Appl. No.: **19,066**

**Related U.S. Application Data**

[63] Continuation-in-part of Ser. No. 576,849, Sept. 2, 1966, abandoned.

[52] U.S. Cl. .... **260/400, 252/8.7, 117/139.5**

[51] Int. Cl. .... **C07c 143/90, C11d 1/28**

[58] Field of Search.... **260/400**

[56]

**References Cited**

**UNITED STATES PATENTS**

2,734,833 2/1956 Thurston ..... 117/139.5

*Primary Examiner*—Elbert L. Roberts

*Attorney*—Charles J. Fickey

[57]

**ABSTRACT**

Process for producing a novel composition of the class normally employed as softening agents for cotton and rayon textiles during hot finishing treatments, and storage of the composition. More particularly, the invention relates to the alkali metal salts of sulfonated bisfumarates of the mixed glycerides of unsaturated fatty acids, having at least 15 percent by weight of polyunsaturated fatty acids therein.

**3 Claims, No Drawings**

## **NON-YELLOWING SOFTENING AGENT FOR COTTON AND RAYON TEXTILES**

This application is a continuation-in-part of co-pending application, Ser. No. 576,849, filed Sept. 2, 1966 now abandoned.

This invention relates to a novel process for producing a novel composition of the class normally employed as softening agents for cotton and rayon textiles during hot finishing treatments, and storage of the composition. More particularly, the invention relates to the alkali metal and ammonium salts of bis-esters of sulfosuccinic acid and glycerides of hydroxy-containing, unsaturated higher fatty acids. The invention also relates to cellulosic and cellulosic containing substrates, such as toweling, having a high affinity for water, i.e., good rewetability, after impregnating with the novel softening composition.

Prior compositions and process of making those compositions, such as typically disclosed in U. S. Pat. No. 2,734,833, (1) require fatty acid radicals to be derived from animal and vegetable oils and fats with no substantial amounts of hydroxy acids and having less than 15 percent by weight of polyunsaturated fatty acids therein, or in which the unsaturation is reduced to below the 15 percent, and (2) require heat treatment of the monoglyceride in the presence of at least 10 mole percent of added fatty acid such as stearic acid, palmitic acid, oleic acid, etc., to prevent the formation of insoluble resins believed to be cross-linked glycerol-fumaric (or glycerolmaleic)

esters. Thus, prior art processes fall within specific limitations as to the nature of the fatty acid which may be employed, and require specific process limitations such as those described above, in order to obtain a satisfactory product. Moreover, the products of the prior art processes, such as those discussed above, are softeners which, when applied to cellulosic or cellulosic-containing substrates such as textile materials, provide a final product which has a reduced affinity for water, i.e., which does not have good rewettability.

In addition to the above limitations of prior processes, it should be noted that the prior art processes were expensive because of a large number of steps required, the higher tem-

substrates such as toweling, for example, unless a surface active agent which imparts rewettability were added to the prior art softening agent, however, this substantially reduced the handle imparted by the softening agent.

It is an object of this invention to obtain a softening agent for cotton and rayon textiles and blends thereof having high quality handle and having good rewettability.

Another object is to obtain a softening agent which is a liquid.

Another object is to obtain a softener agent which is cold water soluble.

Another object is to provide a process for producing said product which process is more economical as a result of fewer critical steps, temperatures, and reaction times required.

Another object is to obtain a finishing agent composition which when employed on textile cellulosic material such as cotton and rayon textiles does not impart an undesirable yellowing of the fabric subsequent to the finishing thereof.

Other objects become apparent from the above and following disclosure.

The objects of this invention are obtained by a novel composition described below, the process of making the composition, and celluloses impregnated with the composition.

The novel composition of this invention comprises a metal or ammonium salt of a sulfosuccinate-type bis-ester of a monoglyceride of a hydroxy-containing, unsaturated higher fatty acid. The bis-ester is believed to have the following general structural formula:



wherein R is a ricinoleoyl group, R<sup>1</sup> is hydrogen or lower alkyl, M is an ammonium or alkali metal cation, (e.g., sodium, potassium, etc.) and n<sub>1</sub> and n<sub>2</sub> are each an integer from 0 to 2, where the sum of n<sub>1</sub> and n<sub>2</sub> is at least 1 to about 3.

The term "hydroxy-containing unsaturated hydrocarbons" is

The term "hydroxy-containing, unsaturated higher fatty acid" includes acids such as ricinoleic acid and substituted forms thereof, provided the acids are the functional equivalent of ricinoleic acid in the composition of this invention. The fatty acids are hydroxy acids.

A typical composition is the sulfosuccinate of the monoglyceride of ricinoleic acid, of the following formula:



peratures required, and the long periods of reaction required, or combinations of these. In the prior processes, if any of the steps were eliminated, or temperatures or times of reaction were significantly modified, the problem of increased degrees of formation of undesirable cross-linked polymers became more pronounced. Moreover, if cross-linking was avoided, the final softening agent product characteristically required hot water in order to obtain solubility, and the softening agent product itself characteristically was in the form of a solid. Both the property of being solid, and the property of being soluble only in hot water increased the expense of handling and of employing the softening agents in subsequent use on a textile substrate. Additionally, the use of the prior art softening agents on cellulosic or cellulose containing materials resulted in a loss of affinity for water. Therefore, the prior art softening agents were characteristically limited to uses which did not require good rewettability. Accordingly the prior art softening agents characteristically could not be employed on

The major commercially available ricinoleic acid-containing oil is castor oil which normally contains at least about 75 percent ricinoleic acid, and preferably at least about 80 percent, a typical castor oil composition being:

|                       |            |
|-----------------------|------------|
| ricinoleic acid       | 85%        |
| oleic acid            | 8.5%       |
| linoleic acid         | 3.5%       |
| stearic acid          | 0.5 - 2.0% |
| dihydroxystearic acid | 1 - 2%     |

It should be noted that castor oil is the only readily and commercially available oil which contains a "hydroxy fatty acid" as a major component. It is believed that only an unsaturated, hydroxy acid of this type provides the beneficial results of this invention.

The process of preparing the compositions of this invention may be defined as reacting a monoglyceride of a hydroxy-con-

taining, unsaturated higher fatty acid with an unsaturated dibasic aliphatic carboxylic acid or anhydride of the fumaric-acid-type in an amount sufficient to form a bis-ester of said monoglyceride, and sulfonating said bis-ester.

Although the fumaric-type-acid may be any one or more of the fumaric acid series, fumaric acid is the preferred acid to be reacted with the monoglyceride. Other suitable dibasic unsaturated acids include maleic, citraconic, mesaconic, pyrocinchoninic, glutaconic, hydromuconic, and the like.

Although it is not essential that the bis-ester referred to above in the process of this invention be the reaction product resulting from the use of 100 percent pure monoglyceride, the preferred embodiment employs glycerides which are substantially solely the monoglycerides, such as would be obtained by transesterifying a triglyceride of ricinoleic acid, i.e., castor oil, with glycerine in the presence of a catalytic amount of a hydroxide of an alkali metal, employing the triglyceride and the glycerine in relative ratio of from about 1:4 up to about 3:4. However, a mixture of monoglycerides and diglycerides is normally present in the product of such a transesterification, and such a mixture has been found to contain a molar ratio of these two constituents within the range of about 50-95 percent of monoglyceride and about 50-5 percent of diglyceride. It is within the scope of this invention to employ such a mixture.

Characteristically, the ricinoleic acid (the primary component of castor oil) bis-ester is prepared by a two or three step process. If the monoglyceride is already available, it is not necessary to go through the first step. However, the monoglyceride is preferably obtained by the process described in the preceding paragraph. In that process, typical hydroxides include sodium hydroxide, ammonium hydroxide, etc. After a reaction sufficient to form the monoglyceride product, the monoglyceride and unsaturated acid or acid anhydride of the fumaric-acid-type are admixed and condensed sufficiently to obtain a fumaric-acid-type bis-ester. The fumaric-acid-type acid or anhydride may be any acid or acid-anhydride of an acid of the fumaric-acid series including, for example, maleic acid, glutaconic acid, citraconic acid, mesaconic acid, hydromuconic acid, pyrocinchoninic acid, and the like. Preferably, the fumaric-acid-type compound is employed in an amount of at least about one-half mole of fumaric-type acid per mole of the glycerides. The resulting bis-ester is then sulfonated in a conventional manner by refluxing, normally under pressure, in the presence of an aqueous solution of alkaline metal or ammonium bisulfite or metabisulfite whereby the corresponding salt is obtained directly. Also, preferably the sulfonating reaction is carried out in the presence of an alcohol such as isopropyl alcohol.

Salts of other bases may be readily obtained by first acidifying an alcoholic solution of the alkali metal or ammonium salts whereby the free sulfonic acid is obtained, filtering off the inorganic salt of the acid used and reacting the sulfonic acid with the desired base. Although they are not ordinarily employed in textile finishing treatments, salts of the polyvalent metals such as calcium, barium, zinc, lead, cadmium, and the like may be prepared, if desired, by adding stoichiometric quantities of their oxides or hydroxides to the alcoholic sulfosuccinic acid ester solution followed by stirring until the salt formation is complete. Salts of organic bases such as methyl, ethyl, or butyl amine; guanylurea, guanidine; hydroxyethyl-guanidine; biguanide; ethanolamine; triethanolamine; higher aliphatic amines; aromatic amines; heterocyclic bases such as nicotine, pyridine, quinoline; and alkaloids may also be prepared by the same method, as well as by direct sulfonation employing the sulfites and bisulfites of the organic bases.

Some of the advantages of the above composition and process of obtaining the composition are as follows.

The composition of this invention does not require that the unsaturation be reduced to below 15 percent, nor require a low "unsaturation" as would be evidenced by low iodine

value; the ricinoleic acid content of the castor oil approaches about 87 percent (a high concentration) and the ricinoleic acid is highly unsaturated. Similarly the composition of this invention does not require a treatment to prevent the formation of insoluble resin; in contrast to the prior art processes, in the absence of such treatment, there is in the process of this invention no evidence of the formation of an insoluble resin. Moreover, the novel process of this invention of reacting to form the bis-ester of ricinoleic acid, for example, requires less strenuous reaction conditions, i.e., the reaction precedes more smoothly without difficulties at lower reaction temperatures and at shorter periods of time necessary to obtain the final product.

Additionally, the process of this invention has fewer required steps and is more economical in not requiring high reaction temperatures and long periods of time for reaction to take place. The process does not require the "reduction" of "unsaturation" by hydrogenation. There are no difficulties encountered as to any tendency to form insoluble resins during the process.

The softener composition of this invention is easily handled because it is a "liquid", in contrast to the "solid" state of the prior art "tallow" product, for example. The softener composition of this invention is cold-water-soluble, in contrast to the tallow-product of prior art which requires hot water to obtain solubility. The softener composition of this invention imparts to a cellulosic or cellulosic-blend substrate the property of good rewettability, whereby it can be easily and quickly rewet. This is in contrast to the tallow-product, for example, which does not rewet easily nor quickly; good rewettability makes the novel composition of this invention of value for use on toweling, for example.

In employing the novel bis-esters of the invention in textile softening treatments, a dispersion of from about 0.5 percent to about 3 percent or more, based on the weight of the dispersion, of the selected bis-ester is prepared in aqueous medium or, if the textile is to be sized at the same time, in an aqueous size bath. The textile material is thereafter impregnated in the bath to a wet pickup of substantially 100 percent of the weight of fabric and then dried according to normal operating procedure. Ordinarily, where no sizing agent is employed it is unnecessary to have more than about 1 percent of the softening agent on the fabric in order to obtain the desired softness of hand in the product. On the other hand, where a sizing agent is used, it is sometimes necessary to increase the softening agent content to about 3 percent or more to obtain the desired improvement in softness of hand in the treated fabric.

The above-described invention is illustrated in the following example. The example, however, limits this invention only to the extent that such limitations appear in the appended claims.

#### EXAMPLE 1

55 One mole of castor oil (the triglyceride of mainly ricinoleic acid) is transesterified with two moles of glycerine in the presence of a trace of sodium hydroxide, using agitation and elevated temperatures. When this step is complete, xylene is added and the batch is cooled.

60 Fumaric acid (one-half mole of fumaric acid per mole of castor oil mixed glycerides) is added and the bis-ester of the castor oil mixed glycerides is formed, by stripping out water (azeotropic distillation).

65 The bis-ester is sulfonated at reflux, under pressure, in the presence of water, isopropyl alcohol, and sodium bisulfite (one mole sodium bisulfite per mole bis-ester).

70 It is understood that the above-described and illustrated invention is not limited except to the extent of the appended claims. It is within the scope of this invention to include substitutes and equivalences within the scope of the ordinary artisan.

I claim:

1. A metal salt of an ester of the formula:

## BEST AVAILABLE COPY

3,679,719

5



wherein R is a ricinoleyl group, R<sup>1</sup> is selected from the group consisting of hydrogen or lower alkyl, M is a cation selected from the group consisting of ammonium or alkali metal cations, n<sub>1</sub> and n<sub>2</sub> are each integers from 0 to 2, where the sum of

n<sub>1</sub> and n<sub>2</sub> is at least 1 to about 3.

2. A metal salt according to claim 1, in which said cation is sodium.

10 3. A compound of the formula:



\* \* \* \* \*

25

30

35

40

45

50

55

60

65

70

75